

## UNITED STATES PATENT OFFICE

1,939,068

## RECOVERY OF COPPER MINERALS OR VALUES BY FROTH FLOTATION

Reginald John Lemmon, Norton - on - Tees, England, assignor to Imperial Chemical Industries Limited, a corporation of Great Britain

No Drawing. Application June 25, 1931, Serial No. 546,918, and in Great Britain September 3, 1930.

## 1 Claim. (Cl. 209—167)

This invention relates to the recovery of copper minerals or values from copper ores or products containing copper minerals or values, and particularly to the recovery of copper minerals or values from so-called oxidized ores, by which are meant copper ores in which the copper values occur chiefly or to a substantial extent in chemical combination with oxygen. Such oxidized ores, which may or may not include a proportion of copper values in chemical combination with sulphur, have hitherto been difficult to treat by froth flotation processes inasmuch as the copper values are not readily floated by the customary flotation agents.

I have now found that the recovery of copper minerals or values from oxidized copper ores can be greatly improved by the use of a cyanide compound as hereinafter defined, in conjunction with one or more frothing agents, for example the known and commonly used frothing agents, with or without additional substances such as those known in the art as collecting agents, depressing agents, dispersion agents, or conserving agents. The term cyanide compound as used herein and in the appended claim comprises only cyanides of the alkali or alkaline earth metals ammonium cyanide, and hydrocyanic acid itself. Those compounds may either be used as such, or in solution, or as prepared in situ, e. g. by action of hydrocyanic acid upon alkaline compounds present in or added to the ore pulp. If desired more than one such cyanide compound may be employed.

The proportion of cyanide compound used is usually small; it will to some extent be dependent upon the general nature of the ore and the proportion of oxidized or sulphide minerals contained therein, and may be from a fraction of one pound per ton of ore, to two or more pounds (calculated in terms of sodium cyanide), according to the duty it is required to perform. Preferably the proportion of cyanide compound employed is from  $\frac{1}{4}$  to 2 pounds per ton of ore, as we have found that on the whole the best results are obtained within these limits. We have found that recovery is to a certain extent impaired if greater proportions of cyanide compound are employed.

The addition of the cyanide compound may be made to the flotation circuit in various ways,

for example, as one of the reagents introduced into the first or other flotation unit of a froth concentration apparatus, or the addition may be made to the ore pulp in a previous stage of its preparation for flotation recovery, i. e. in the procedure known as "pre-treatment", or in such other manner as a preliminary trial test may show to be the more efficient.

55 60

A quantity of Rhodesian copper ore, containing bornite ( $Cu_2FeS_3$ ), malachite ( $CuCO_3 \cdot Cu(OH)_2$ ), azurite ( $2CuCO_3 \cdot Cu(OH)_2$ ), and chrysocolla ( $CuSiO_3 \cdot 2H_2O$ ), was wet crushed to 80 mesh I. 65 M. M. to form a pulp of 1:5 solid-water ratio, blast furnace creosote being added in the proportion of  $\frac{1}{6}$  pound per ton of ore. The resulting pulp was treated in a sub-aeration flotation machine, with the further addition of cresylic 70 acid in the proportion of  $\frac{1}{6}$  pound per ton of ore. A first froth concentrate was obtained which contained the bulk of the sulphide and silicate copper present in the ore, the actual assays being given below.

75

An addition of sodium cyanide was then made to the pulp, in the proportion of  $\frac{1}{2}$  pound per ton of ore, and a second froth concentrate was obtained which contained the bulk of the ammonium carbonate-soluble copper present in the ore. 80

A further addition of pine oil ( $\frac{1}{6}$  pound per ton of ore) and cresylic acid ( $\frac{1}{2}$  pound per ton of ore) was then made to the pulp and a third froth concentrate obtained which contained the greater part of the residual copper values. 85

The assays of the various concentrates were as follows:—

| Material                | Weight per cent | Total copper per cent | Per cent copper in ore as sulphide and silicate minerals | Per cent copper in ore soluble in ammonium carbonate | 90  |
|-------------------------|-----------------|-----------------------|----------------------------------------------------------|------------------------------------------------------|-----|
| Crude ore.....          | 100.00          | 2.06                  | 0.68                                                     | 1.38                                                 | 95  |
| First concentrate.....  | 1.20            | 40.30                 | 36.93                                                    | 3.37                                                 |     |
| Second concentrate..... | 4.10            | 19.50                 | 2.26                                                     | 17.24                                                |     |
| Third concentrate.....  | 7.10            | 2.98                  | 0.65                                                     | 2.33                                                 |     |
| Tailings.....           | 87.60           | 0.65                  | 0.11                                                     | 0.54                                                 |     |
|                         |                 |                       |                                                          |                                                      | 100 |

The per cent recoveries effected were thus as follows:—

| 5  | Material                | Total copper | Copper in ore as sulphide and silicate minerals | Copper in ore soluble in ammonium carbonate |
|----|-------------------------|--------------|-------------------------------------------------|---------------------------------------------|
| 10 | Crude ore.....          | 100.0        | 100.0                                           | 100.0                                       |
|    | First concentrate.....  | 23.4         | 65.1                                            | 2.9                                         |
|    | Second concentrate..... | 38.7         | 13.6                                            | 51.0                                        |
|    | Third concentrate.....  | 10.2         | 6.8                                             | 11.9                                        |
|    | Tailings.....           | 27.6         | 14.1                                            | 34.1                                        |

- 15 It will be noted that the recovery of total copper before the addition of sodium cyanide was very low, and that the addition of sodium cyanide resulted in the recovery of a substantial amount 20 of the oxidized copper minerals, together with a further amount of copper as sulphide.

*Example 2*

- 25 A quantity of copper ore, containing bornite, malachite, cuprite ( $Cu_2O$ ) and native copper, in a siliceous gangue, was wet-crushed to 80 mesh I. M. M. to form a pulp of 1:5 water-solid ratio, with the addition in grinding of one-eighth of 30 one pound of sodium cyanide, one-quarter of one pound of blast furnace creosote, one-twelfth of one pound of pine oil, all per ton of ore. The resulting pulp was treated in a sub-aeration flotation machine, and a first froth concentrate obtained, assaying as given below. An addition of one-half of one pound of sodium cyanide, one-third of one pound of blast furnace creosote, and one-third of one pound of pine oil, all per ton of ore, was then made in the machine, and a second 40 froth concentrate obtained. The assays of the two concentrates and tailings were as follows:—

| 45 | Material                | Weight per cent | Total copper per cent | Per cent copper soluble in ammonium carbonate |
|----|-------------------------|-----------------|-----------------------|-----------------------------------------------|
| 50 | Crude ore.....          | 100.0           | 3.60                  | 3.36                                          |
|    | First concentrate.....  | 1.0             | 30.67                 | 26.49                                         |
|    | Second concentrate..... | 16.0            | 16.60                 | 15.75                                         |
|    | Tailings.....           | 83.0            | 0.77                  | 0.70                                          |

- 55 The per cent recoveries effected were thus as follows:—

| 60 | Materials               | Total copper | Copper soluble in ammonium carbonate |
|----|-------------------------|--------------|--------------------------------------|
| 65 | Crude ore.....          | 100.0        | 100.0                                |
|    | First concentrate.....  | 8.5          | 7.8                                  |
|    | Second concentrate..... | 73.6         | 75.0                                 |
|    | Tailings.....           | 17.9         | 17.2                                 |

- 70 By way of comparison with the above procedure, the following results were obtained by froth concentration without the use of cyanide:—A similar sample of ore to that employed above was wet-ground to 80 mesh I. M. M. to form a pulp of 1:5 water-solid ratio, with the addition in grinding of one-quarter of one pound of

blast furnace creosote and one-twelfth of one pound of pine oil, both per ton of ore. The resulting pulp was treated in a sub-aeration flotation machine and a first froth concentrate obtained, assaying as given below. An addition of one-third of a pound of pine oil, and one-third of a pound of blast furnace creosote, both per ton of ore, was then made in the machine, and a further froth concentrate obtained. The assays of the two concentrates and tailings were

80

85

15 The per cent recoveries effected were thus as follows:—

| Material                | Weight per cent | Total copper per cent | Per cent copper soluble in ammonium carbonate |
|-------------------------|-----------------|-----------------------|-----------------------------------------------|
| Crude ore.....          | 100.0           | 3.26                  | 2.95                                          |
| First concentrate.....  | 2.0             | 23.65                 | 19.18                                         |
| Second concentrate..... | 3.25            | 15.11                 | 13.14                                         |
| Tailings.....           | 94.75           | 2.43                  | 2.26                                          |

90

95

20 It will be noted that poor recoveries were obtained both in the case of the total copper (including bornite) and also in the case of the soluble copper constituent.

115

25 From the above figures it will be observed that the addition of sodium cyanide had a marked influence upon both the flotation of the total and soluble copper in the pulp, resulting in the substantial recoveries, severally, of 82.1 per cent total copper, and 82.8 per cent soluble copper. Corresponding recoveries without sodium cyanide were 29.5 per cent total copper and 27.4 per cent soluble copper.

120

30 In the case of minerals such as those treated in the above examples, which contain both sulphide and oxidized ore, it is preferred to perform a preliminary flotation without cyanide, or with a relatively small quantity of the same, for the purpose of removing the bulk of the relatively easily floated sulphide and to float the remaining oxidized ore with the aid of a cyanide compound as described.

125

35 I am aware that in the froth concentration of mixed sulphide ores containing iron sulphide the addition of cyanide has been suggested for the purpose of effecting differential flotation of the sulphides through the depressing action of the cyanide upon the flotation of iron sulphide, but the present invention makes use of an entirely different principle, namely the efficiency of cyanide compounds as reagents whereby oxidized copper minerals or compounds, not otherwise readily floated, are rendered amenable to froth flotation.

135

40 Various changes may be made in the method of carrying out my invention and I do not desire to be limited to the procedure hereinbefore set out, except as defined in the following claim.

140

145

150

I claim:

A process for the recovery of copper values from copper ores in which the values occur both in chemical combination with oxygen and as sulphide, said ores being substantially free from gold or silver, which comprises subjecting the crushed ore to froth concentration in stages in

the first of which principally the sulphide values are separated, no cyanide compound being present, while in a succeeding stage a cyanide compound is added to the pulp, which enhances the flotability of the oxidized copper compounds.

80

REGINALD JOHN LEMMON.

10

85

15

90

20

95

25

100

30

105

35

110

40

115

45

120

50

125